

# United States Patent

Benford et al.

[15] 3,644,185

[45] Feb. 22, 1972

- [54] **METHOD OF IMPROVING MAGNETIC PERMEABILITY OF CUBE-ON-EDGE ORIENTED, SILICON-IRON SHEET STOCK**

- [72] Inventors: **James G. Benford**, Monroeville Boro; **Edward B. Stanley**, Washington Township, Westmoreland, both of Pa.

- [73] Assignee: **United States Steel Corporation**

- [22] Filed: Nov. 10, 1969

- [21] Appl. No.: 875,562

- [52] U.S. Cl..... 204/140.5, 148/110, 148/112,  
204/140

- [51] Int. Cl. .... C23b 1/00, C23b 3/06  
[58] Field of Search ..... 204/140, 140.5

- [58] **Field of Search** ..... 204, 248, 270, 283

[56]

## References Cited

UNITED STATES PATENTS

- |           |         |                   |           |
|-----------|---------|-------------------|-----------|
| 2,479,302 | 8/1949  | Bondley .....     | 204/140.5 |
| 3,223,602 | 12/1965 | Wawrousek .....   | 204/140.5 |
| 3,413,204 | 11/1968 | Rexer et al. .... | 204/140.5 |
| 2,820,003 | 1/1958  | Logan et al. .... | 204/140.5 |
| 2,334,699 | 11/1943 | Faust .....       | 204/140.5 |

*Primary Examiner*—John H. Mack

*Assistant Examiner—T. Tufariello*

Attorney—Forest C. Sexton

[57]

## ABSTRACT

The method of improving the magnetic properties of conventional cube-on-edge oriented, silicon-iron sheet stock by providing the sheet with a light electropolish before or after the final high-temperature orientation anneal sufficient to substantially eliminate large microscopic peaks but insufficient to significantly enhance average surface smoothness.

**4 Claims, No Drawings**

**METHOD OF IMPROVING MAGNETIC PERMEABILITY  
OF CUBE-ON-EDGE ORIENTED, SILICON-IRON SHEET  
STOCK**

**BACKGROUND OF THE INVENTION**

Recent advancements in the electrical steel art have revealed a new approach to improving the magnetic properties of ferromagnetic materials, such as silicon-iron sheet stock, showing that surface smoothness is a substantial factor in the materials magnetic permeability. Specifically, it has been shown that permeability can be enhanced for a given sheet material if the surface has a smoothness of about 5 microinches or smoother. To this end, pertinent publications teach cold reducing the sheet with very smooth rolls to effect the surface smoothness of 5 microinches or less. For example, see U.S. Pat. No. 3,347,718. Although this procedure is successful in providing an improved permeability, the process is expensive because such extreme smoothnesses are not easily maintained on the work rolls of commercial rolling mills, 20 requiring greatly increased roll maintenance costs.

**SUMMARY OF THE INVENTION**

This invention is predicated upon our discovery that an exceptionally light electropolish on the surface of conventional cube-on-edge grain oriented, silicon-iron sheet stock not only improves magnetic permeability by a very limited polishing action, but contributes to texture development to enhance the desired grain orientation. In this process, extreme smoothness of the finished sheet is not desired since optimum results are obtained at average smoothnesses of about 8-18 microinches which is not substantially smoother than commercial oriented sheet now on the market. It is apparent that substantially less power is necessary to achieve this light polish as compared to an excessive polish down to a smoothness of 5 microinches.

It is therefore an object of this invention to provide an improved cube-on-edge grain-oriented, silicon-iron sheet stock having an enhanced orientation and magnetic permeability.

It is another object of this invention to provide a method for improving the magnetic permeability of conventional cube-on-edge grain-oriented, silicon-iron sheet stock wherein the sheet is given an exceptionally light electropolish which, although not substantially increasing average surface smoothness, does increase magnetic permeability and preferred orientation.

**DESCRIPTION OF THE PREFERRED EMBODIMENT**

The starting material used in the process of this invention is a conventional intermediate silicon steel containing from 2.5 to 3.5 percent silicon, which has been processed by conventional procedures for a cube-on-edge grain-oriented silicon-iron sheet. Typical composition objectives for such a steel are substantially as follows:

|            |                 |
|------------|-----------------|
| Silicon    | 2.5 to 3.5%     |
| Carbon     | at least 0.010% |
| Sulfur     | at least 0.010% |
| Manganese  | 0.06 to 0.12%   |
| Phosphorus | up to 0.010%    |
| Nitrogen   | up to 0.010%    |

The cold rolling procedures utilized in the process of this invention may be substantially the same as those used in the prior art. That is, the hot rolled band, having a thickness of about 0.08 inch, is first cleaned to remove mill scale and then cold rolled to final gage, i.e., 0.011 to 0.014 inch, usually in two cold reductions with intermediate annealing. The procedures we refer to are well known to those skilled in the art.

Although we find the above cold rolling procedure to be ideally suited to this process, other two or three step cold reductions may be used. More important than the number of cold reductions and the extents thereof is that after each cold reduction the sheet must be annealed not only to relieve internal stresses induced by the cold working, but more impor-

tantly to effect a fine grained primary recrystallization structure development prior to the final anneal. Although batch annealing may be used in place of continuous annealing, we prefer continuous annealing because it provides more uniform heating and allows a faster annealing cycle to minimize exaggerated grain growth. We therefore prefer our intermediate anneals to be continuous anneals at temperatures within the range 1,400° to 1,700° F. in a protective atmosphere. The annealing time must be sufficient to completely effect primary recrystallization. Prolonged heating, however, should be avoided so that grain growth is minimized. If batch annealing is used, it is advisable to avoid temperatures in excess of 1,750° F. to eliminate the possibility of extensive grain growth.

Decarburization is usually effected during the last intermediate anneal to reduce the carbon content of the sheet to levels of 0.004 percent or less. For optimum results we prefer to anneal at a temperature within the range 1,400° to 1,550° F., or ideally at about 1,475° F. for a period of about 3 to 5 minutes in a moist atmosphere containing hydrogen having a dew point of +70° F.

As in other prior art processes, the sheet is given a final high temperature anneal after the cold rolling and intermediate annealing steps. This final high temperature anneal, or orientation anneal, is preferably a box anneal at a temperature of from 2,000° to 2,150° F. which effects a secondary recrystallization yielding the desired oriented grains. The annealing time which may vary from 1 to 35 hours, must, of course, be sufficient to effect complete secondary recrystallization (grain orientation) and sulfur removal. As expected, the annealing time required is inversely proportional to annealing temperature so that higher temperatures will require shorter annealing times.

The above procedures are substantially like those frequently practiced in the prior art. The crux of this invention resides in a step whereby the sheet is given a light electropolish either before or after the final high temperature anneal. Optimum results are achieved if the electropolishing is effected before the final anneal. Electropolishing may be performed either in a batch process or continuous process in accordance with well known electropolishing procedures. For example, a suitable light polish can easily be effected in a period of 2 to 3 minutes in a chromic acid-phosphoric acid bath at a current density of 310 amp./ft.<sup>2</sup>. The electropolishing time can of course be reduced by using higher current densities.

The primary objective of the electropolishing step is not only to effect a slightly smoother surface, but also to properly condition the sheet surface to effect better texture development during the secondary recrystallization. In order to derive the benefit of this later objective, it is obviously necessary that the sheet be electropolished prior to the high temperature final anneal wherein grain orientation is effected. In this regard, the electropolish serves to remove any surface or near surface oxides that might interfere with the secondary recrystallization process either by obstructing the motion of grain boundaries or by serving as sources of oxygen potential that might unfavorably alter the surface energy relationships of grains of various orientations.

Although optimum results can be achieved only if the sheet is electropolished prior to the final anneal as explained above, some of the benefits of this invention can be realized by electropolishing the oriented sheet after the final anneal. Since the sheet has already undergone secondary recrystallization after the final anneal, the electropolishing can no longer enhance orientation as described above, but it can nevertheless provide a smoother surface on the final product which will improve magnetic permeability.

Whether the sheet is electropolished before or after the final anneal, it is not essential or even desirable that exceptionally smooth surfaces be achieved. In fact, optimum results are achieved at surface smoothnesses of about 8 to 20 microinches, which is not necessarily smoother than the surfaces of unpolished sheets. The electropolishing will neverthe-

less provide significant improvements in magnetic permeability with little or no actual change in average roughness. To be more specific, commercially produced oriented sheets seldom have average roughnesses above about 20 microinches, and typically have average roughnesses in the range 10 to 20 microinches. After the light electropolish of this invention, the sheets may still have average roughnesses in the 8 to 20 microinch range, but yet have substantially improved magnetic permeability. It is obvious therefore that our electropolishing step does provide benefits other than those normally expected from merely rendering a smoother surface.

To explain the above phenomenon, we have learned that magnetic permeability is not so much a function of surface smoothness, but more importantly is a function of the large microscopic peaks which are usually randomly dispersed over the surface of cold rolled sheet steels. The larger such peaks and the greater their number, the lower the sheet's magnetic permeability will be. Hence, our electropolishing treatment may not and need not actually change the average sheet roughness as measured by a "Surfindicator," but it will eliminate or reduce the large microscopic peaks. Although excessive electropolishing to produce a substantially smoother surface does also eliminate such peaks, this also removes substantial amounts of surface metal unnecessarily which serves only to reduce recovery and efficiency without any improvement in permeability.

It is apparent, therefore, that in our process all that is required is that the sheet be subjected to a light electropolish regardless of the average surface roughness before or after the polish. It follows that a sheet electropolished according to this invention will have a higher magnetic permeability than will a like sheet not so polished even though the nonpolished sheet

0.018 percent sulfur, and 3.26 percent silicon. All samples were identically processed to 0.012-inch thick oriented sheet substantially as described above except that samples 2 were electropolished after the high temperature final anneal whereas samples 1 were not electropolished. Electropolishing of samples 2 were effected for 2 minutes in a chromic acid-phosphoric acid bath 100 grams chromic acid and 532 ml. phosphoric at a current density of 310 amp./ft.<sup>2</sup> and at 25 volts. No measurements of surface roughness were made because the magnesium silicate glass formed on the fully processed material precluded a meaningful measurement.

TABLE I

| Samples | Average Permeability |                   |        |        |        |
|---------|----------------------|-------------------|--------|--------|--------|
|         | No.                  | Surface Treatment | 10 kg. | 15 kg. | 17 kg. |
| 1       | Not Electropolished  | 32661             | 25846  | 8925   |        |
| 2       | Electropolished      | 36576             | 29152  | 9146   |        |

Table II below is substantially the same as Table I except that for these tests, the electropolishing was performed prior to the high temperature anneal. The chemistry of these heats and the electropolishing procedures were identical to those shown above. Roughness measurements were made on these samples since both had essentially clean surfaces. Magnetic-torque measurements on the nonelectropolished samples revealed 86 percent texture development, whereas, the electropolished samples were developed to 92 percent.

TABLE II

| Samples | Surface roughness      |                   |                                  | Average permeability               |        |        |        |        |
|---------|------------------------|-------------------|----------------------------------|------------------------------------|--------|--------|--------|--------|
|         | No.                    | Surface treatment | Arithmetic average (microinches) | Peaks per inch over 50 microinches | 10 kg. | 15 kg. | 17 kg. |        |
| 3.....  | Not electropolished... |                   | 11-13                            |                                    | 286    | 31,500 | 27,778 | 9,197  |
| 4.....  | Electropolished.....   |                   | 8-11                             |                                    | 71     | 34,187 | 32,061 | 14,295 |

may have a smoother surface.

The electropolishing procedures themselves may be substantially the same as those known and practiced in the prior art. Although any person skilled in the art could therefore readily determine a variety of suitable electropolishing parameters, we have been most successful with a chromic acid-phosphoric acid bath at current densities within the range 300 to 1,000 amp./ft.<sup>2</sup>. Within this range we have preferred a current density of about 440 amp./ft.<sup>2</sup> at polishing times of from 30 to 120 seconds, with optimum results at about 120 seconds. For example, a given heat of steel was processed to grain oriented sheet without any electropolishing and had a magnetic permeability of 9,200 at 17 kilogauss. An identical sheet electropolished for 30 seconds at 440 amp./ft.<sup>2</sup> prior to the final anneal, but otherwise identically processed had a magnetic permeability of 11,500 at 17 kilogauss. Extending the electropolish to 120 seconds resulted in a magnetic permeability of 12,700 at 17 kilogauss. An average roughness of 10 to 13 microinches was not appreciably changed by either electropolish. Extending the electropolish beyond 120 seconds did not appreciably effect permeability but merely resulted in excessive metal removal.

Tables I and II below are presented to better illustrate the detailed advantages of this invention. Table I shows the average improvement in magnetic permeability values for a given heat of oriented sheet at 10, 15 and 17 KG. The heat shown in Table I had the following chemistry: 0.022 percent carbon, 0.08 percent manganese, 0.006 percent phosphorus,

From the above tables, it will be readily apparent to those skilled in the art that the process of this invention is capable of producing cube-on-edge grain oriented, silicon-iron sheet stock having an improved magnetic permeability.

We claim:

1. A method for increasing the magnetic permeability of conventional cube-on-edge grain oriented silicon-iron sheet stock containing from 2.5 to 3.5 percent silicon comprising lightly electropolishing the sheet surfaces sufficient to substantially eliminate large microscopic peaks, but insufficient to appreciably enhance average surface smoothness to thereby render a surface smoothness of from 8 to 20 microinches.
2. In the method for producing cube-on-edge grain oriented silicon-iron sheet stock wherein a steel containing 2.5 to 3.5 percent silicon is cold reduced to 0.011 to 0.014 inch in a series of cold rolls with intermediate annealing to effect primary recrystallization following each cold roll, and finally annealing at high temperatures to effect secondary recrystallization orientation, the improvement comprising electropolishing the sheet surfaces after cold rolling sufficient to substantially eliminate large microscopic peaks, but insufficient to appreciably enhance average surface smoothness.
3. The method of claim 2 in which said electropolishing is performed before the final high-temperature anneal.
4. The method of claim 2 in which said electropolishing is performed after the final high-temperature anneal.

\* \* \* \* \*